

April 18, 1933.

M. L. BEGEMAN

1,904,118

MANUFACTURE OF WIRE GLASS

Filed May 14, 1931

FIG.1.



FIG.2.



INVENTOR

MYRON L. BEGEMAN

BY HIS ATTORNEYS

*Cooper, Kerr & Dunham*

Patented Apr. 18, 1933

1,904,118

# UNITED STATES PATENT OFFICE

MYRON L. BEGEMAN, OF ST. LOUIS, MISSOURI, ASSIGNOR TO MISSISSIPPI GLASS COMPANY, OF NEW YORK, N. Y., A CORPORATION OF NEW YORK

## MANUFACTURE OF WIRE GLASS

Application filed May 14, 1931. Serial No. 537,370.

This invention pertains to the manufacture of wire glass by the process of forming a first half-sheet, laying the reinforcing wire on that first half-sheet, and then welding the 5 second half-sheet thereon.

It has been customary to form the two half-sheets between pairs of rolls, but that process has not been satisfactory on account of the fact that the rolls chill the sheets to 10 a certain extent, forming a skin or film on the sheet surfaces so that when the two half-sheets are brought together it is difficult to get a perfect weld between the half-sheets.

If a sheet (or half-sheet) be formed between a roll and a non-rotatable member, the 15 surface formed by the gate is not chilled, therefore no skin forms on that surface and it welds easily.

In my application Serial No. 364,754, filed 20 May 21, 1929, of which this application is a continuation in part, apparatus is shown for forming half-sheets between rolls and gates and then welding the two half-sheets together, the weld taking place between the 25 surfaces formed by the non-rotatable members.

It has been found that, under certain conditions, good welds may be obtained between half-sheets when only one of the contacting 30 surfaces is formed by a rotatable member, and the principal object of the present invention is to disclose apparatus and method for forming sheets in that manner.

Further and other objects and advantages 35 will be apparent from the specification and claims, and from the accompanying drawing which illustrates what is now considered the preferred embodiment of the invention.

Fig. 1 shows in cross-section apparatus 40 for forming one half-sheet between rolls, the other half-sheet between a roll and a gate, with a pair of rolls for welding the two half-sheets together.

Fig. 2 shows in cross-section a modification in which one half-sheet is formed between rolls and the other half-sheet is formed between the welding rolls, the gate serving to control the flow of metal which forms the second half-sheet.

50 In the drawing, molten metal 10 flows

over furnace lips 12 and 14 onto the upper surfaces of rolls 16 and 18. Above roll 18 (Fig. 1) is an adjustable roll 20, to form between those rolls a pass in which the half-sheet 22 is formed. Above roll 16 is an 55 adjustable gate 17, the lower edge of which is set near roll 16 to form therebetween a pass in which the half-sheet 24 is formed. The two half-sheets are carried by their respective lower rolls through the pass 60 formed between rolls 16 and 18 where the half-sheets are welded together to form the finished sheet 26. The half-sheet 24 contains enough heat to break down the film on half-sheet 22 and thereby permit the half-sheets 65 to properly weld together. Any slight surplus of metal forms a ball 28 between rolls 16 and 18, and serves to compensate for any irregularities in the thickness of the half-sheets.

In Fig. 2, a half-sheet 22 is formed, as before, between rolls 18 and 20, but gate 17, instead of forming a pass between itself and roll 16, is moved away from that roll to simply control the position of the metal that 70 forms the second half-sheet. In this modification there is a sufficient mass of metal 75 over the point where the finished sheet is formed to overcome the chill on the first-sheet and thereby insure a good weld in the final forming pass between rolls 16 and 18. The body of molten metal serves also to take 80 care of any irregularities in thickness of the rolled half-sheet.

In case it is desired to have reinforcing 85 wire in the finished sheet, the wire 30 is fed, past guide rollers 32 to rest on the surface of the first half-sheet, upon which it rides through the final roll pass to emerge in the middle of the finished sheet 26.

It is to be understood that the invention is not limited to the specific embodiment herein illustrated and described but may be used in other ways without departure from its spirit as defined by the following claims.

I claim:

1. In apparatus for making glass, a pair of forming rolls, means for feeding molten metal between said rolls to form a half-sheet, means comprising a roll and a non-rotatable 100

member adjacent thereto and with said roll forming a pass to produce a second half-sheet, and means for welding said half-sheets to form a single sheet.

- 5 2. In apparatus for making sheet glass, a pair of rolls, means for feeding molten metal onto each of said rolls, a roll adjacent one of said pairs of rolls for controlling the flow of metal thereover, a non-rotatable member adjacent the other of said pair of rolls and with the other of said rolls forming a pass for controlling the flow of metal thereover, and means for subsequently passing the metal from both rolls simultaneously through a sheet-forming pass to weld them into a single sheet.
- 10 3. The invention set forth in claim 2 in which said sheet forming pass comprises the space between said pair of rolls.
- 15 4. The invention set forth in claim 1 in which means is provided for guiding reinforcing wire between said half-sheets whereby said wire is embedded in the finished sheet.
- 20 5. The invention set forth in claim 2 in which means is provided for guiding reinforcing wire through said forming pass whereby said wire is embedded in the finished sheet.
- 25 33. In testimony whereof I hereto affix my signature.

MYRON L. BEGEMAN.

35

40

45

50

55

60

65